

Patented July 27, 1926.

1,594,185

# UNITED STATES PATENT OFFICE.

SAMUEL A. NEIDICH, OF EDGEWATER PARK, NEW JERSEY.

## METHOD OF AND MEANS FOR TREATING FILAMENTS FORMED FROM VISCOSE.

No Drawing.

Application filed May 23, 1925. Serial No. 32,455.

Liquid viscose (cellulose sulphocarbonate) may be coagulated or precipitated to form a gelatinous semi-solid cellulose hydrate complex by progressively projecting a stream 5 of such viscose into a heated atmosphere or into an aqueous solution containing a suitable acid, for instance, sulphuric or hydrochloric acid, or containing an acid salt such as sodium bi-sulphite or ammonium chloride either with or without neutral salts or dehydrators, or both.

Such a filament is amorphous and so soft and impressionable that it is easily deformed even by contact with itself in successive 15 convolutions, and even slight indentations of the ultimate commercial filament formed by drying and contraction from its primarily soft gelatinous form are conspicuously noticeable because of the reflection of light 20 therefrom, whereas; the commercial value of such filament is largely dependent upon its uniformity of cross section and uniformly lustrous appearance. Consequently, when it is desired to form such filaments of uniform 25 cross section free from indentation, it is undesirable to wind them in the usual way upon the surface of bobbins or other similar containers, and a method of dropping such filaments in bulk is desirable. However, 30 when such filaments are dropped in loose bulk, even their own weight impressing the upper layers upon the lower layers, produces such indentations as to be undesirable.

Therefore, it is the object and effect of 35 my invention to provide means to suspend and support such filaments practically continuously from the time they leave the coagulating bath until they are sufficiently firm to resist such deformation or indentation, 40 so that the final product is of uniform cross section and without the defects aforesaid and consequently of greater commercial value.

To that end my invention includes the 45 provision of means to prevent adjacent layers of the filament from thus marking each other by their weight, by supporting that weight in a liquid of approximately equal specific gravity. Such liquid is preferably 50 one which is also capable of rendering the filament sufficiently firm to be self-supporting without deformation. For instance, an aqueous solution containing six and one half per cent of sodium bi-sulphite, three per 55 cent of sodium sulphate (Glauber's salt),

and four per cent of  $\text{NH}_4\text{CL}$  (salammoniac) supports such filaments and simultaneously renders them firm enough to be self-supporting. However, the specific gravity may be varied by increasing or decreasing the 60 amount of salt in the solution.

I have found by experiment that by permitting the precipitated filaments to drop in a mass in the above solution and remain still for several hours, they are sufficiently firm 65 to undergo the chemical treatment described in my copending application serial No. 26825 filed April 29, 1925.

The flotation liquid above specified is varied in specific gravity from 1.04 to 1.20 70 in accordance with variations in the specific gravity of the filament being suspended therein, which varies in specific gravity in accordance with the character of the means employed for its coagulation and the stage 75 of the latter. Moreover although an ordinary coagulating bath consisting of an aqueous solution of sulphuric acid ( $\text{H}_2\text{SO}_4$ ) ranges from 1.2 to 1.5 specific gravity it 80 has a tendency to increase in gravity constantly because of the formation therein of sodium sulphate incident to the reactions involved in the coagulating process. Therefore, to attain the best flotation effect above contemplated, constant care must be exercised to maintain the specific gravity of the flotation liquid substantially uniform in 85 compensation for its tendency to increase in gravity, as the upward pressure upon the filament from a flotation liquid which is too 90 heavy may produce marks upon the filament as detrimental as the marks produced by downward pressure. Consequently, it is essential to the attainment of the full benefit of my invention to maintain the flotation 95 liquid of approximately the same specific gravity as the filament being suspended therein, despite variations in the specific gravity of such filament.

A typical example of the use of my invention to form an artificial horseshair filament is as follows: Liquid viscose is forced, conveniently by a pump or air pressure, through a single hole about .025 inch in diameter into a coagulating bath including an 100 aqueous solution of sodium bi-sulphite and ammonium chloride which promptly coagulate the viscose to an impure cellulose hydrate complex sufficiently coherent to be mechanically drawn through and from such 110

bath over a roller. Such filament, being isolated in its passage through such bath, is of uniform circular cross section and free from the defects aforesaid as it is discharged by said roller. However, to thus continue to support it in isolated position would be impracticable for lack of space and consequent consideration of cost of manufacture etc. Therefore, I provide a container into which such filament may gravitate and in which it may be supported, in mass, by flotation, as above contemplated, and preferably in a bath containing chemicals which facilitate the formation of the initially soft and gelatinous substance of the filament to the desired solid resilient state. However, the flotation liquid may also contain any suitable solute substantially chemically inert with reference to the filament but affecting the normal specific gravity of the liquid; for instance, glucose or molasses. Such containers may be circular in plan and oscillated at such slow rate that the filament is piled in circumferentially successive convolutions around the axis of rotation of the container; the latter being oscillated rather than revolved, to avoid twisting the filament. Such oscillation is preferably progressive, being alternately to a greater arcual extent in one direction than in the other, so that the container is ultimately charged with a mass of filament entirely surrounding its axis with the overlapped portions of the filament progressively circumferentially distributed therein and supported by the gravitational flotation effect of the liquid in the container. However, the filaments thus discharged as above contemplated from the coagulating bath may be received in a suitable container of rectangular configuration progressed transversely to the axis of said discharging roller beneath the latter; the region of discharge of the filament from the roller being progressively changed from end to end of the latter by guiding the filament to the roller through a device which is correspondingly reciprocated, with the effect of piling the filament in such rectangular container in convolutions which are first transversely and second longitudinally successive with reference to the length of such container, in which the filaments may be supported by the gravitational flotation effect of the liquid as aforesaid. As above contemplated; in the course of manufacture by any ordinary means, such filaments are successively immersed in liquids which are normally of different specific gravities; beginning with a chemical coagulating bath and successive chemical purifying and aqueous washing baths; while the filament is progressively increasing in specific gravity; but each bath in which the filament is successively received may have its

normal specific gravity so modified, in accordance with my invention, as to support the filament therein, as above described.

Therefore, I do not desire to limit myself to the precise details of construction, arrangement or procedure herein set forth, as it is obvious that various modifications may be made therein without departing from the essential features of my invention, as defined in the appended claims.

I claim:

1. The method of treating a filament formed from viscose which consists in supporting it in mass in a liquid of specific gravity substantially the same as that of the filament.

2. The method of treating a filament formed from viscose which consists in subjecting it in mass to the action of a liquid coagulant normally of greater specific gravity than the filament but which has been modified by inclusion of an element decreasing its specific gravity until the latter is substantially the same as that of the filament.

3. The method of treating a filament formed from viscose which includes supporting it in mass by flotation suspension in a liquid, the specific gravity of which is approximately as great as that of the filament.

4. The method of treating a filament formed from viscose which includes supporting it in mass by flotation in a liquid, the specific gravity of which is substantially the same as that of the filament; and containing a chemical capable of acting upon the filament.

5. The method of treating a filament formed from viscose which includes supporting it in mass by flotation in a liquid, the specific gravity of which is substantially the same as that of the filament, and containing a chemical capable of acting upon the filament, and a substance substantially chemically inert with reference to the filament but affecting the specific gravity of the liquid.

6. The method of treating a filament formed from viscose which includes supporting the latter in mass in a liquid containing an aqueous solution of a substance capable of modifying the specific gravity of the solution in correspondence with the specific gravity of the filament to suspend the latter.

7. The method of treating a filament formed from viscose which consists in suspending the latter in mass in a liquid of such specific gravity as to balance the gravitational effect upon the filament and thus suspend the latter in said liquid.

8. Means for treating in mass a filament formed from viscose which includes a liquid vehicle for said filament of specific gravity approximately as great as that of the filament.

9. Means for treating in mass a filament formed from viscose which includes a liquid coagulant for said filament normally of greater specific gravity than the filament but which has been modified by inclusion of an element decreasing its specific gravity until the latter is substantially the same as that of the filament. 45
10. Means for treating in mass a filament formed from viscose which includes a filament flotation liquid, the specific gravity of which is approximately as great as that of the filament. 50
11. Means for treating in mass a filament formed from viscose which includes a filament flotation liquid, the specific gravity of which is approximately as great as that of the filament; and containing a chemical capable of acting upon the filament. 55
12. Means for treating in mass a filament formed from viscose which includes a filament flotation liquid, the specific gravity of which is approximately as great as that of the filament, and containing a chemical capable of acting upon the filament, and a substance substantially chemically inert with reference to the filament but affecting the specific gravity of the liquid. 60
13. Means for treating in mass a filament formed from viscose which includes liquid containing an aqueous solution of a substance capable of modifying the specific gravity of the solution in correspondence with the specific gravity of the filament to suspend the latter. 65
14. Means for treating in mass a filament formed from viscose which consists of a liquid of such specific gravity as to balance the gravitational effect upon the filament and thus suspend the latter in said liquid. 70
15. Means for treating in mass a filament formed from viscose which includes an aqueous solution, the specific gravity of which is rendered approximately as great as that of the filament. 75
16. Means for treating in mass a filament formed from viscose which includes an aqueous solution, the specific gravity of which is approximately as great as that of the filament; and containing a chemical capable of acting upon the filament. 80
17. Means for treating in mass a filament formed from viscose which includes a liquid, the specific gravity of which is substantially the same as that of the filament, and containing a chemical capable of acting upon the filament, and a solute substantially chemically inert with reference to the filament but affecting the normal specific gravity of the liquid. 85
18. Means for treating in mass a filament formed from viscose which includes a liquid containing a solute modifying the normal specific gravity of the solution in correspondence with the specific gravity of the filament to suspend the latter. 90
19. Means for treating in mass a filament formed from viscose which includes a liquid, the specific gravity of which is approximately as great as that of the filament, and containing a chemical capable of acting upon the filament, and a solute affecting the normal specific gravity of the liquid. 95
20. Means for treating in mass a filament formed from viscose which includes a liquid containing an aqueous solution of a substance modifying the specific gravity of the solution in correspondence with the specific gravity of the filament to suspend the latter. 100

In testimony whereof, I have hereunto signed my name at Burlington, New Jersey this 20th day of May, 1925.

SAMUEL A. NEIDICH.